

Patented July 7, 1953

2,644,788

# UNITED STATES PATENT OFFICE

2,644,788

## ELECTRODEPOSITION OF NICKEL

Wilbur J. Shenk, Jr., Shaker Heights, Ohio, assignor to The Harshaw Chemical Company, Cleveland, Ohio, a corporation of Ohio

No Drawing. Application March 31, 1951,  
Serial No. 218,693

6 Claims. (Cl. 204—49)

1

This invention relates to electrodeposition of metals, and more specifically to a process of, and solutions for, use in a process of electrodepositing nickel, characterized in that the resulting nickel electrodeposit is bright as it comes from the plating solution, is very ductile and very smooth. More particularly, the present invention has to do with the discovery of cooperating addition agents suitable for use in an aqueous, acid, nickel plating solution, and having the capability of producing electrodeposits of unusual brilliance on comparatively rough surfaces accompanied by extreme ductility and increase in smoothness over the base metal.

Many of the so-called bright plating solutions are capable of producing deposits of extreme brilliance when the deposit is made on very highly polished base metal, such as polished brass, but produce less impressive deposits on rougher surfaces, such as steel or brass, which has been buffed with abrasive leaving a surface which has some sheen but is not highly polished. It is an object of the present invention to provide a solution capable of producing deposits of full brightness on surfaces which are less than fully polished as will be indicated on a quantitative basis hereinafter. It is a further object to produce deposits which are extremely ductile and which, on base surfaces of some degree of roughness, are smoother than the base metal itself; that is, the deposit builds smoothness rather than becoming less smooth with increasing thickness as is the case with some bright deposits.

I have now discovered that the foregoing objects can be attained in surprising degree by the use in an aqueous, acid, nickel plating solution made up essentially of a nickel electrolyte of the class consisting of nickel sulfate, nickel chloride, and mixtures of nickel sulfate with nickel chloride, and an effective amount of each of two cooperating addition agents, one of such addition agents being selected from the class consisting of compounds represented by the formula:



and salts and hydrates thereof,  $n$  being an integer from 1 to 3, where R represents a radical selected from the class consisting of hydrogen, chlorine, bromine, methyl, ethyl, propyl, butyl, cyclohexyl, isopropyl, and phenyl, and R' represents a radical selected from the class consisting of hy-

drogen, chlorine, bromine, methyl, ethyl, propyl, butyl, cyclohexyl, isopropyl, and phenyl, and where R and R', taken together, represent a bivalent radical selected from the class consisting of methylidene, ethylidene, propylidene, isopropylidene, and butylidene; for example:

- (a) 1-(carboxymethyl) pyridinium chloride,  
(b) 1-(carboxymethyl) pyridinium bromide,  
(c) 1-(1'-carboxyamyl) pyridinium bromide,  
(d) 1-(1'-carboxypropyl) pyridinium bromide,  
(e) 1-(1'-carboxyl-1'phenylmethyl) pyridinium bromide,  
(f) 1-(1'-carboxyethyl) pyridinium chloride,  
(g) 1-(1'-carboxyvinyl) pyridinium bromide,  
(h) 1-(2'-carboxyethyl) pyridinium chloride,  
(i) 1-(2'-carboxypropyl) pyridinium chloride,  
(j) 1-(1'-carboxyisobutyl) pyridinium bromide,  
(k) 1-(1'-carboxybutyl) pyridinium bromide,  
(l) 1-(3'-carboxypropyl) pyridinium bromide.

The second of said addition agents is an aromatic sulfur compound containing at least one aromatic ring of the benzene (single ring) or naphthalene type to which is attached an  $\text{SO}_2\text{R}$  group where R is hydroxy or  $\text{NH}_2$ . Preferably such second said addition agent is a compound of the formula:



or



where R is selected from the class consisting of  $\text{OH}$ ,  $\text{NH}_2$ ,  $\text{NHSO}_2\text{Ph}$ ,  $\text{NHSO}_2\text{alkyl}$  (1 to 12 carbon atoms), chloro and bromo substitution products, and nickel, iron, cobalt, sodium, and potassium salts of the foregoing as well as saccharine and its corresponding salts.

Examples of these addition agents are as follows:

45

### 1. Dibenzene sulfonamide



### 2. N-ethane sulfonyl benzene sulfonamide



50

55

3

### 3. Saccharine



#### 4. Benzene sulfonic acid



## 5. Benzene sulfonamide



The nickel, iron, cobalt, sodium, and potassium salts of the foregoing are substantially equivalent and can be used with equally good results.

It will be seen that the addition agents of the first-mentioned type are pyridinium carboxylate compounds having one or more carbon atoms interposed between the nitrogen atom of the pyridinium radical and the carboxy group. Substitution in the side chain can be made freely as indicated, whereas substitution on the pyridinium ring appears to impair the usefulness of the compound. The quaternary nitrogen atom is the essential point of attachment of the side chain.

As will be seen, the addition agents of the second-mentioned class are sulfonates, sulfonamides, sulfonimides, and sulfonic acids having one or more aromatic rings of the benzene type, that is, having a single-ring or benzene nucleus. Substitutions may be made on the ring of various groups such as alkyl (1 to 12 carbon atoms), halogen (chlorine, bromine), and the like.

Addition agents of the pyridinium carboxylate type are employed in concentration of the order of 0.1 to 1.0 gram per liter while the addition agents of the second class are employed in concentrations of the order of .5 to 2.5 grams per liter.

It is to be understood that all statements made herein concerning the capabilities of the addition agents presuppose the use of one, or a mixture of two or more, from each class; that is, one or more of the pyridinium carboxylate compounds together with one or more of the aromatic sulfur compounds. For convenience the pyridinium carboxylate compounds are considered to be brighteners, and the aromatic sulfur compounds are considered to be carriers or auxiliary brighteners, although actually they are cooperating brighteners and either may be regarded as auxiliary to the other.

4

The constituents of the bath according to the preferred practice of invention are: (1) water, (2) nickel sulfate, nickel chloride, or nickel sulfate with nickel chloride, (3) an aromatic sulfur compound of the class defined such as benzene sulfonate, soluble saccharine, dibenzene sulfonamide, or the like, and a pyridinium carboxylate compound of the class defined. An additional ingredient of the solution which is desirable is a buffering agent such as boric acid, formic acid, or the like. It will be noted that in respect to major constituents, the solutions are similar to the well-known "all-sulfate," "all-chloride," and "sulfate-chloride," or Watts type nickel plating solutions.

The preferred basic solutions in connection with which the invention is realized are as follows:

### All sulfate

|                                              |                                                |
|----------------------------------------------|------------------------------------------------|
| NiSO <sub>4</sub> ·7H <sub>2</sub> O         | 100 to 400 gms., preferably<br>200 to 300 gms. |
| Boric acid                                   | 0 to 60 gms., preferably<br>10 to 40 gms.      |
| Wetting agent (e. g. sodium lauryl sulfate). | 0 to 5 gms., preferably 0.5<br>to 1 gm.        |
| H <sub>2</sub> O to make                     | 1000 cc.                                       |

### All chloride

|                                              |                                            |
|----------------------------------------------|--------------------------------------------|
| NiCl <sub>2</sub> ·6H <sub>2</sub> O         | 50 to 250 gms., preferably 100 to 200 gms. |
| Boric acid                                   | 0 to 60 gms., preferably 10 to 40 gms.     |
| Wetting agent (e. g. sodium lauryl sulfate). | 0 to 5 gms., preferably 0.5 to 1.0 gm.     |
| H <sub>2</sub> O to make                     | 1000 cc.                                   |

### Sulfate-chloride (Watts Type)

|                                              |                                                |
|----------------------------------------------|------------------------------------------------|
| NISO <sub>4</sub> ·7H <sub>2</sub> O         | 100 to 400 gms., preferably<br>200 to 300 gms. |
| NiCl <sub>2</sub> ·6H <sub>2</sub> O         | 10 to 60 gms., preferably<br>25 to 40 gms.     |
| Boric acid                                   | 0 to 50 gms., preferably<br>15 to 40 gms.      |
| Wetting agent (e. g. sodium lauryl sulfate). | 0.5 to 5 gms., preferably<br>0.5 to 1 gm.      |

To each of the foregoing basic solutions I add a suitable quantity of each, or a mixture of two or more of each, of the two cooperating addition agents. One of said addition agents or mixtures is one of the aromatic sulfur type, and the other is of the pyridinium carboxylate type, both described above. The solution may contain an anti-pit agent although the deposits usually will be suitable for many purposes without any other addition agent for eliminating the pitting. Sodium lauryl sulfate may be used as an anti-pit agent, although, as stated, its use is not ordinarily essential, and other wetting agents or mixtures of wetting agents may be used for control of pitting.

The following specific examples will serve to illustrate the invention:

Having thus described my invention, what I claim is:

1. A method of electrodepositing nickel on a metallic surface in the form of a deposit which is bright as taken from the plating solution without further treatment, and which deposit is ductile and smoother than said metallic surface when the root mean square average deviation of the irregularities in the surface thereof from the average surface plane is about 10 to 15 microinches, and the thickness of the deposit is about 0.001", which method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being a pyridinium carboxylate compound selected from the class consisting of 1-(carboxymethyl) pyridinium chloride, 1-(carboxymethyl) pyridinium bromide, 1-(1'-carboxyamyl) pyridinium bromide, 1-(1'-carboxypropyl) pyridinium bromide, 1-(1'-carboxy-1'-phenylmethyl) pyridinium bromide, 1-(1'-carboxyethyl) pyridinium chloride, 1-(1'-carboxyvinyl) pyridinium bromide, 1-(2'-carboxyethyl) pyridinium chloride, 1-(2'-carboxypropyl) pyridinium chloride, 1-(1'-carboxyisobutyl) pyridinium bromide, 1-(1'-carboxybutyl) pyridinium bromide, and 1-(3'-carboxypropyl) pyridinium bromide, and the second of said addition agents being an aromatic sulfur compound selected from the group consisting of compounds of the formula  $ArSO_2R$ , where Ar is selected from the class consisting of benzene and naphthalene radicals and R is selected from the class consisting of OH, NH<sub>2</sub>,  $NHSO_2Ph$ ,  $NHSO_2$  alkyl wherein the alkyl group contains from 1 to 12 carbon atoms, and chloro and bromo substitution products of said compounds and the nickel, iron, cobalt, sodium and potassium salts of the foregoing.

2. A method of electrodepositing nickel on a metallic surface in the form of a deposit which is bright as taken from the plating solution without further treatment, and which is ductile and smoother than said metallic surface when the root mean square average deviation of the irregularities in the surface thereof from the average surface plane is about 10 to 15 microinches, and the thickness of the deposit is about 0.001", which method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being 1-(carboxymethyl) pyridinium chloride and being present in concentration from 0.1 to 1.0 gram per liter, and the other of said addition agents being dibenzene sulfonamide and being present in concentration from 0.5 to 2.5 grams per liter.

3. A method of electrodepositing nickel on a metallic surface in the form of a deposit which is bright as taken from the plating solution without further treatment and which is ductile and smoother than said metallic surface when the root mean square average deviation of the irregularities in the surface thereof from the average surface plane is about 10 to 15 microinches, and the thickness of the deposit is about 0.001", which

method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being 1-(1'-carboxyvinyl) pyridinium chloride and being present in concentration from 0.1 to 1.0 gram per liter, and the other of said addition agents being dibenzene sulfonamide and being present in concentration from 0.5 to 2.5 grams per liter.

4. A method of electrodepositing nickel on a metallic surface in the form of a deposit which is bright as taken from the plating solution without further treatment, and which is ductile and smoother than said metallic surface when the root mean square average deviation of the irregularities in the surface thereof from the average surface plane is about 10 to 15 microinches, and the thickness of the deposit is about 0.001", which method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being 1-(1'-carboxyethyl) pyridinium chloride and being present in concentration from 0.1 to 1.0 gram per liter, and the other of said addition agents being dibenzene sulfonamide and being present in concentration from 0.5 to 2.5 grams per liter.

5. A method of electrodepositing nickel on a metallic surface in the form of a deposit which is bright as taken from the plating solution without further treatment, and which is ductile and smoother than said metallic surface when the root mean square average deviation of the irregularities in the surface thereof from the average surface plane is about 10 to 15 microinches, and the thickness of the deposit is about 0.001", which method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being 1-(2'-carboxyethyl) pyridinium chloride and being present in concentration from 0.1 to 1.0 gram per liter, and the other of said addition agents being dibenzene sulfonamide and being present in concentration from 0.5 to 2.5 grams per liter.

6. A method of electrodepositing nickel on a metallic surface in the form of a deposit which is bright as taken from the plating solution without further treatment, and which is ductile and smoother than said metallic surface when the root mean square average deviation of the irregularities in the surface thereof from the average surface plane is about 10 to 15 microinches, and the thickness of the deposit is about 0.001", which method comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness and smoothing power as aforesaid, one of said addition agents being 1-(carboxymethyl) pyridinium chloride and being present in concentration from

0.1 to 1.0 gram per liter, and the other of said addition agents being saccharine and being present in concentration from 0.5 to 2.5 grams per liter.

WILBUR J. SHENK, Jr.

References Cited in the file of this patent

UNITED STATES PATENTS

| Number    | Name        | Date         |
|-----------|-------------|--------------|
| 2,315,802 | Lind et al. | Apr. 6, 1943 |

| Number    | Name  | Date          |
|-----------|-------|---------------|
| 2,513,280 | Brown | July 4, 1950  |
| 2,550,449 | Brown | Apr. 24, 1951 |

OTHER REFERENCES

|                                                         |
|---------------------------------------------------------|
| Raub et al., Metal Finishing, August 1940, pp. 429-432. |
| Silman, Metal Industry, November 24, 1944, pp. 330-332. |